

July 16, 1929.

H. SKALL

1,721,475

WORK REST BLADE FOR CENTERLESS GRINDERS

Filed Feb. 6, 1928

FIG. 1.



FIG. 2.



INVENTOR:

HAROLD SKALL,

By Robert Burns

ATTY.

## UNITED STATES PATENT OFFICE.

HAROLD SKALL, OF CHICAGO, ILLINOIS, ASSIGNOR TO DANLY MACHINE SPECIALTIES, INC., OF CHICAGO, ILLINOIS, A CORPORATION OF ILLINOIS.

## WORK-REST BLADE FOR CENTERLESS GRINDERS.

Application filed February 6, 1928. Serial No. 252,169.

This invention relates more particularly to the type of centerless grinders in which the grinding operation is performed by the perimeter of the grinding wheel and the 5 present improvement has for its object:

To provide a structural formation of a work support or blade for centerless grinders of the type above mentioned, embodying the feature of a maximum durability, efficiency and economy in production, all as 10 will hereinafter more fully appear.

In the accompanying drawing:

Fig. 1 is an end elevation, partly in section, embodying a mechanical arrangement 15 and structural formation of the invention.

Fig. 2 is a side elevation of the preferred form of the work supporting blade.

Like reference numerals indicate like 20 parts in both views.

As shown in Fig. 1 of the drawing, the centerless grinder mechanism comprises in the main, a downwardly and rapidly rotating grinding wheel 1, and an upwardly and slowly rotating feeder or regulating wheel 25 2, with the movement of the peripheries of the two wheels in opposite directions where they contact with the work, adapted to impart a turning movement to such work during the grinding operation. The work being

30 supported in proper position by the usual work rest or blade 3, carried in an adjustable manner is a fixed supporting post 4, with the top face of the blade 3 in proper operative relation to a line drawn between the centers of the wheels 1 and 2 aforesaid.

Previous to this invention work supports or blades of the type above described, were formed with a main body portion of cheaper metal with the work supporting face of the

40 blade formed of a strip of steel alloy, welded to said main body portion and having the required degree of wear resisting hardness. Such form of work supporting blade was subject to considerable wear in continued

45 use and was open to the farther serious objection that particles of the metallic article operated on and of the grinding wheel, released in actual use, had a tendency to adhere to and "hill" upon the top surface of a

support or blade, with a tendency to score 50 and render imperfect the surface of the article at the end of a grinding operation.

With a view to remove such difficulties and produce a superior work support or blade of the present type, I have found after 55 extended experiments, changes and practical tests during such experiments, that cast iron, preferably in the form of an iron alloy hereinafter described, will when its work supporting surface is chilled to a moderate 60 depth, provide in a ready and economical manner, a work support or blade having a much greater life than the much more expensive work supports heretofore used and referred to above, and with an almost entire 65 absence of an accumulation or hillng of the ground particles on its supporting face, above referred to, as an objectionable feature in the former type of work supports.

The principal alloying elements in the 70 present iron alloy, above referred to, are manganese, silicon and carbon, with a small percentage of phosphorus, sulphur and combined carbon and chromium. The proportions of which may be slightly varied within 75 limits given in the following table and by which superior results are obtained:

|                  | Per cent.    |
|------------------|--------------|
| Silicon -----    | 1.50 to 1.75 |
| Manganese -----  | .50 to .70   |
| Phosphorus ----- | .25 to .35   |
| Sulphur -----    | Max. .10     |
| Carbon -----     | 2.50 to 2.75 |
| Combination :    |              |
| Carbon -----     | .40 to .60   |
| Chromium -----   | Max. .20     |

The remainder iron.

Work rests or supporting blades made from alloyed iron containing materials in the proportions specified in the above table, and 90 after the resting or supporting face 3' of the support or blade 3 formed therefrom has been chilled in an ordinary manner to a depth approximately three-quarters of an inch, and a hardness of at least 50 Rockwell 95 C numerals, possesses in a superior degree the desired wear resisting qualities and hardness above set forth.

Having fully described my invention, what I claim and desire to secure by Letters Patent, is:—

5 A wear resisting work supporting blade for centerless grinders, comprising a cast metal alloy of iron, carbon, silicon, manganese, phosphorus, and chromium, the supporting face of the blade having a chill of

some depth with a hardness of at least 50 Rockwell C numerals and a chill face of a 10 natural smooth and dense nature adapted to resist deposit and piling up of grindings in actual use.

In testimony whereof I hereunto affix my signature.

HAROLD SKALL.